

United States Patent [19]  
Haller, Jr.

[11] 3,953,203  
[45] Apr. 27, 1976

[54] JEWELRY ALLOYS

[75] Inventor: Mitchell W. Haller, Jr., York, Pa.  
[73] Assignee: Dentsply Research & Development Corporation, Milford, Del.  
[22] Filed: Jan. 24, 1975  
[21] Appl. No.: 543,751

[52] U.S. Cl. .... 75/171; 75/134 B;  
75/134 F; 75/134 M  
[51] Int. Cl.<sup>2</sup> ..... C22C 19/05  
[58] Field of Search ..... 75/170, 171, 134 B,  
75/134 F, 134 M; 148/32, 32.5

[56]

References Cited

UNITED STATES PATENTS

|           |         |                     |        |
|-----------|---------|---------------------|--------|
| 2,628,900 | 2/1953  | Jackson et al. .... | 75/171 |
| 3,841,868 | 10/1974 | Dudek et al. ....   | 75/171 |

Primary Examiner—R. Dean

[57]

ABSTRACT

A base metal alloy primarily for jewelry use comprising a major portion of nickel and minor proportions selected from the group tin, chromium, silicon, aluminum, niobium and manganese.

8 Claims, No Drawings

## JEWELRY ALLOYS

CROSS-REFERENCE TO RELATED  
APPLICATIONS

U.S. Pat. application Ser. No. 472,787, filed May 23, 1974, by Charles R. Manning and Mitchell W. Haller for Dental Alloy.

## BACKGROUND

This invention relates to base metal alloys having particular utility for jewelry applications.

In particular, a major object of the present invention is to provide a base metal alloy to be used as an alternative to so-called white gold in jewelry applications.

In order to provide a suitable alloy capable for jewelry applications, certain characteristics should be present:

- a. A melting temperature low enough to permit casting in gypsum investments while retaining compatibility with phosphate and other higher temperature investments.
- b. Ability to obtain accurate casting detail.
- c. Sufficient ductility in castings to allow "stretching" or changes in size of rings and other jewelry pieces.
- d. Ability to solder.
- e. Corrosion resistance.
- f. Non-irritability to skin.
- g. Ability to maintain a shine and to be polished.

The alloys of the present invention include the foregoing characteristics in addition to others which render them superior material for use in the manufacture of jewelry.

DESCRIPTION OF THE PREFERRED  
EMBODIMENTS

The present invention relates to metal alloys primarily useful for jewelry applications.

The alloys of the present invention are designed as alternatives to the use of gold, so-called white gold, or other noble metals, without loss of desirable qualities.

The alloys of the present invention comprise a major portion of nickel with lesser amounts of other elements as are useful to impart the properties required for jewelry use.

Polishability and the ability to maintain a shine are, of course, properties essential in a jewelry alloy. In this connection, it is important to provide an alloy which is carbon-free or essentially so, since the presence of more than about 0.1% carbon will seriously impair polishability and ductility. It is important that the carbon content be maintained below 0.1% and preferably below 0.03%.

Similarly, ductility is an important quality in jewelry alloys. The use of tin and/or manganese assists in lowering the melting range while still allowing the alloy to have sufficient ductility. The use of manganese is recommended in the approximate range of from 20 to 50%, and tin in the approximate range of from 2 to 8%. However, where non-noble metals are used, a skillful blending of components is required. For example, if excessive amounts of tin are used (above about 9% in the present case) the alloy will become brittle, and lose ductility. As mentioned, the presence of carbon in amounts over 0.1% will adversely affect ductility.

Corrosion resistance is an important factor also. Here, chromium appears to perform an important function. Thus, unless some other corrosion resistant ele-

ment is used, chromium should be about 8% of the alloy. However, if more than about 18% of the alloy is chromium, there will be an undesirable loss of ductility and higher than desirable melting temperatures will be required.

The jewelry is made, generally, by casting, usually into gypsum or phosphate investment molds. Thus, the melting temperature of the alloy must be sufficiently low (e.g. about 1900°- 2400°F) for casting in gypsum investments. In this regard, tin assists in the lowering of the melting temperature. Specifically, if the alloy contains less than about 2 - 3% tin, the temperature will be too high (unless another temperature suppressing component is used). As stated, however, the use of tin must be regulated, since the inclusion of more than about 8% tin will result in a loss of ductility.

Silicon, it has been found, is a useful ingredient for jewelry alloys since, when used in the range of up to about 1%, it enhances the soldering qualities of the material. In addition, silicon acts as a "scavenger", i.e. it neutralizes impurities, and thus promotes castability. The element also tends to maintain a lower melting temperature.

Aluminum, which may be used up to about 3%, also acts as a scavenger, assists castability and enhances a desirable melting temperature. Aluminum appears to promote the ability of the alloy to withstand elongation without failure, as does manganese.

Nickel is the base material of the alloys of the present invention. This material melts at approximately 2650°F, is compatible with most investments materials, has good ductility and good corrosion resistance.

The first, preferred general group of jewelry alloys of the present invention preferably contain the following ingredients (ranges approximate):

|           |         |
|-----------|---------|
| Tin:      | 2 - 8%  |
| Chromium: | 8 - 18% |
| Silicon:  | 0 - 1%  |
| Aluminum: | 0 - 3%  |
| Niobium:  | 0 - 10% |
| Nickel:   | Balance |

The alloy compositions herein disclosed characteristically have a melting range of from about 1900°F to about 2400°F, an ultimate strength over 70,000 psi, a yield strength of over 52,000 psi, an elongation of over 5%, and a casting temperature within the capability of natural gas-oxygen torches.

The initial alloy preparation is typically carried under an argon cover employing an induction furnace, with the following order of addition of component elements. First, nickel in the form of chips, and chromium in the form of irregularly shaped granules are each weighed out in the appropriate amounts for the composition of alloy being prepared, and thereafter, placed in a crucible. The nickel and chromium components are then dispersed within a zirconia-lined crucible and melted to form a uniform aggregate mixture. An argon cover is maintained over the crucible throughout the melting. The crucible preferably is ceramic and the mixing implements quartz to prevent carbon pick-up. As previously indicated carbon should be kept below 0.1% and preferably below 0.03%.

It should be noted that the quality of all components is important in order to realize and maintain the ductility and elongation properties achievable with these particular alloy compositions.

While the uniform aggregate mixture of nickel and chromium is molten in a homogeneous liquid dispersion, the appropriate weights of silicon and niobium, are prepared for addition to the nickel-chromium melt. The silicon is preferably added in granular form, and the niobium, if used, is added in whatever appropriate form is available. This second group of components is introduced to the crucible within the furnace containing the nickel/chromium homogeneous liquid melt dispersion to form a homogeneous liquid melt mass.

The appropriate amount of tin, in elemental or pre-loyed form is weighed out and added last to the melt. The tin is allowed to disperse as a liquid component within the liquid melt alloy mass to form the homogeneous alloy composition of the present invention. In connection with a second type of alloys of the present invention, manganese may be added to the melt in addition to tin. This melt can then be cast directly into investment molds of gypsum or phosphate, or can be cast into convenient shapes for later re-melting and casting into the desired shapes.

It is important in the preparation of the alloys that oxidation of components, particularly the tin, be minimized in order to adequately control the compositions of the melt. For this reason, initial preparation of the alloy composition is conducted under an argon cover, thereby reducing oxidation and consequent slag formation which would have undesirable effects on the alloy.

Likewise, as indicated, it is important that control of the carbon content of the alloys of the present invention be exercised since objectionable amounts of carbon into the alloy will degrade some of the desired properties. Preferably the alloy should not contain more than 0.1% by weight carbon.

Utilization of the alloy of the present invention in place of gold or gold alloys should not require any additional or different investment materials, casting equipment, or any significant change in technique other than that which is currently employed in a reasonably well equipped jewelry manufacturing facility as used and carried out by reasonably skilled and competent personnel. Likewise, no special handling is required in the use of the alloy of the present invention as such might be required in the use of an alloy which contained Beryllium.

The following examples illustrate alloy compositions of the first, preferred group and their percentages, by weight, of the total composition when made in accordance with the method set forth hereinbefore:

|  |          | EXAMPLE 1 | Percentages |
|--|----------|-----------|-------------|
|  | Nickel   | 79.0      |             |
|  | Chromium | 15.0      |             |
|  | Tin      | 5.0       |             |
|  | Silicon  | 1.0       |             |

|  |          | EXAMPLE 2 | Percentages |
|--|----------|-----------|-------------|
|  | Nickel   | 84.8      |             |
|  | Chromium | 10.0      |             |
|  | Tin      | 5.0       |             |
|  | Aluminum | 0.2       |             |

|  |          | EXAMPLE 3 | Percentages |
|--|----------|-----------|-------------|
|  | Nickel   | 83.8      |             |
|  | Chromium | 10.0      |             |
|  | Tin      | 6.0       |             |
|  | Silicon  | 0.2       |             |

|  |          | EXAMPLE 4 | Percentages |
|--|----------|-----------|-------------|
|  | Nickel   | 84.8      |             |
|  | Chromium | 10.0      |             |
|  | Tin      | 5.0       |             |
|  | Silicon  | 0.2       |             |

-continued  
Percentages

| EXAMPLE 1 |          |
|-----------|----------|
| EXAMPLE 5 |          |
|           | Nickel   |
|           | Chromium |
|           | Tin      |
|           | Niobium  |

82.5  
9.0  
5.0  
3.5

10 The alloys of Examples 1 – 5 melt in the range 2100° – 2400°F, and prove excellent for jewelry use, having good casting characteristics, substantial ductility, can be soldered and pass the standard corrosion tests of a jewelry manufacturer.

15 A second general group of alloys has been discovered which also possess useful qualities for jewelry applications, although the first group described above is preferable. The second group is of the following type:

|    |            |                              |
|----|------------|------------------------------|
| 20 | Manganese: | 20 – 50%                     |
|    | Chromium:  | 8 – 20%                      |
|    | Silicon:   | 0 – 1%                       |
|    | Aluminum:  | 0 – 3%                       |
|    | Nickel:    | Balance                      |
|    | Tin        | also be used, where desired. |

25 Specific examples of the second type are as follows:

| EXAMPLE 6 |           | Percentages |
|-----------|-----------|-------------|
|           | Nickel    | 69          |
|           | Chromium  | 10          |
|           | Tin       | 5           |
|           | Manganese | 15          |
|           | Silicon   | 1           |

  

| EXAMPLE 7 |           | Percentages |
|-----------|-----------|-------------|
|           | Nickel    | 70.9        |
|           | Chromium  | 8.0         |
|           | Tin       | 5.0         |
|           | Manganese | 16.0        |
|           | Aluminum  | 0.1         |

30 35 40 These compositions have a relatively low melting range with the liquidus temperature being below 2200°F are very ductile and can be soldered. Generally, the alloys are acceptable for jewelry use, having the other characteristics, as described above, desirable for such use.

45 50 This invention has been described with reference to the preferred embodiments of the invention. However, the contemplated breadth of the compositions and their applications should be interpreted in light of the specification and claims to include further embodiments which employ equivalent materials for their stated function in the melt and finished alloy.

I claim:

1. An alloy having utility for fabrication into jewelry consisting essentially by weight:

|  |          | Approximate Ranges |
|--|----------|--------------------|
|  | Tin      | 2 – 8%             |
|  | Chromium | 8 – 18%            |
|  | Silicon  | 0 – 1%             |
|  | Aluminum | 0 – 3%             |
|  | Niobium  | 0 – 10%            |
|  | Nickel   | Balance.           |

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6

| Percentages |      |
|-------------|------|
| Nickel      | 79.0 |
| Chromium    | 15.0 |
| Tin         | 5.0  |
| Silicon     | 1.0. |

3. An alloy having utility for fabrication into jewelry consisting essentially by weight:

|          |      |
|----------|------|
| Nickel   | 84.8 |
| Chromium | 10.0 |
| Tin      | 5.0  |
| Aluminum | 0.2. |

4. An alloy having utility for fabrication into jewelry consisting essentially by weight:

Percentages

|          |      |
|----------|------|
| Nickel   | 83.8 |
| Chromium | 10.0 |
| Tin      | 6.0  |
| Silicon  | 0.2. |

5. An alloy having utility for fabrication into jewelry consisting essentially by weight:

|          |      |
|----------|------|
| Nickel   | 84.8 |
| Chromium | 10.0 |
| Tin      | 5.0  |

5 6. An alloy having utility for fabrication into jewelry consisting essentially by weight:

|          |      |
|----------|------|
| Nickel   | 82.5 |
| Chromium | 9.0  |
| Tin      | 5.0  |
| Niobium  | 3.5. |

10 7. An alloy having utility for fabrication into jewelry consisting essentially by weight:

| Percentages |     |
|-------------|-----|
| Nickel      | 69  |
| Chromium    | 10  |
| Tin         | 5   |
| Silicon     | 1   |
| Manganese   | 15. |

15 8. An alloy having utility for fabrication into jewelry consisting essentially by weight:

|           |      |
|-----------|------|
| Nickel    | 70.9 |
| Chromium  | 8.0  |
| Tin       | 5.0  |
| Manganese | 16.0 |
| Aluminum  | 0.1. |

\* \* \* \* \*